

C. M. GAGE, JR.  
PROCESS OF COATING PAPER.  
APPLICATION FILED NOV. 12, 1915.

1,282,564.

Patented Oct. 22, 1918.



Inventor:  
Charles M. Gage, Jr.  
by *Frank Smith & Associates*

Atty's.

# UNITED STATES PATENT OFFICE.

CHARLES M. GAGE, JR., OF EAST PEPPERELL, MASSACHUSETTS.

## PROCESS OF COATING PAPER.

1,282,564.

Specification of Letters Patent. Patented Oct. 22, 1918.

Application filed November 12, 1915. Serial No. 61,182.

*To all whom it may concern:*

Be it known that I, CHARLES M. GAGE, Jr., a citizen of the United States, residing at East Pepperell, county of Middlesex, State 5 of Massachusetts, have invented an Improvement in Processes of Coating Paper, of which the following description, in connection with the accompanying drawing, is a specification, like characters on the drawing 10 representing like parts.

This invention relates to a process for coating paper and has for its object to provide a novel process by which paper can be provided with a superior finish. The ordinary 15 method employed in providing paper, such as is used in printing books, catalogues, etc., with a hard, glazed, smooth surface is to pass the paper through a bath of coating material which is preferably some clay compound, and then pass the coated paper 20 through squeeze rolls which determine the amount of coating to be left on the paper and then subject the paper to the action of brushes which operate on the coated surface 25 thereof and have for their purpose to spread the coating evenly. The paper is then dried in some suitable way and subsequently subjected to the calendering operation to give the surface the final polish.

Sometimes the paper is given a second 30 coating of the finishing material so as to provide a better surface, but so far as I am aware, the second coating has always been applied after the paper has been dried so that the application of the second coating involves the same manipulation of the paper 35 as the application of the first coating does. The placing of two coatings on the paper thus doubles the labor and cost involved in 40 applying one coating and correspondingly increases the cost of manufacture.

My invention comprehends a novel 45 method by which a second coating can be applied to the paper at the same time that the first coating is being applied, thus avoiding the necessity of a double manipulation of the paper and the consequent added labor cost.

In accordance with my method the two 50 coatings can be applied to the paper thereby giving it a superior finish at substantially the same labor cost as that involved in ap-

plying a single coating to the paper. In carrying out my invention I apply a primary coating of finishing material to the 5 paper, preferably by passing the paper through a bath, and then I pass the paper through squeeze rolls which determine the amount of coating to remain on the paper and also operate to force the coating more 60 or less into the pores of the paper and thus fill the surface thereon. The paper is then subjected to the action of usual brushes by which the coating is evened up on the surface and the paper is then subjected to a 65 drying action sufficient to partially dry the coating. The paper is then acted upon for the purpose of still further evening up the coating that is applied thereto so as to prevent any wavy formation in the coating 70 which might be due to the shrinkage of the paper in the drying operation. I then apply the second or finishing coating to the surface of the paper by means of a spray and in such a way that the second coating is 75 evenly applied over the smooth primary coating. By using a spray for applying the second coating it is possible to apply a second coating of any desired thickness and to apply it absolutely uniformly over the surface of the paper. The second coating is then subjected to a brushing action and the paper may then be passed to the usual suction apron and onto the usual drying apparatus where it is completely dried. With 80 my invention it is possible to apply the second coating during the same run as that in which the first coating is applied so that the application of the two coatings does not consume any more time than the usual operation of applying a single coating.

In order to give an understanding of my invention I have illustrated in the drawings diagrammatically an apparatus by which the method may be carried out, but I wish to 85 state that the invention is not limited to the apparatus shown.

In the drawing the paper to be treated is indicated at 1 and is shown as being taken from a roll 2. 3 is a bath of coating material 100 through which the paper 1 is passed. This may conveniently be done by passing the paper over a direction roll 4 down into the bath and around a roll 5. 6 designates

squeeze rolls between which the paper is passed as it leaves the bath. The purpose of these squeeze rolls is to gage the amount of coating which is applied to the paper and 5 also to press the coating material into the pores of the surface of the paper. 7 indicates usual brushes which act on the coated surface of the paper and which are reciprocated or vibrated in different directions for 10 the purpose of evening the coating. Where the paper is coated on both sides, as shown in the drawings, these brushes will be placed to act on both sides of the paper.

The device as thus far described is such 15 as is commonly used in coating paper.

From the brushes 7 the coated paper passes to a drying apparatus which partially dries the paper. This drying apparatus may conveniently be a plurality of 20 nozzles 8 arranged to blow heated air against the paper and where the nozzles are situated on both sides of the paper as shown in the drawing, the paper will be floated between the nozzles and subjected to the drying 25 action of the air currents issuing from the nozzles. This drying of the paper sometimes shrinks it slightly with the result that the coating will have a more or less wavy formation which would be detrimental to 30 perfect printing. To correct this I pass the paper while under slight tension over rolls 9 and 10 which are constructed with a perfectly smooth true surface and which are rotated with a surface speed exactly corresponding 35 to the speed of the paper. These rolls eliminate or correct any wavy formation in the paper and insure that the paper as it leaves the rolls will be perfectly true and evenly coated. A second coating of coating 40 material is then applied to the partially-dried paper by means of a spray, and for this purpose spray nozzles 11 are shown. These spray nozzles may be of any suitable construction and are adapted to spray an even coating of material onto one or both 45 sides of the paper as desired, and they may be regulated to spray a coating of any desired thickness. This second coating is not pressed into the pores of the paper as the 50 first coating is, but merely lies on the surface of the paper and is subjected to the action of a single brush 12 to assist in an even deposit of the coating. From the brush the paper passes to the usual suction apron 13 55 and then into a drying apparatus of any usual formation where it is hung in festoons 14 and subjected to the drying action. After the paper is dried it may be calendered and treated in the usual way. It will be noted 60 that in my improved process both the primary and the secondary or finishing coating is applied to the paper during the same run, thus obviating any separate manipulation of the paper. The advantage of this is that a

single manipulation of the paper suffices for 6 the application of both coatings, and, therefore, both the labor cost and time involved in applying the second coating is negligible.

It will also be noted that the second coating 7 is merely applied to the surface of the paper and is not forced into the pores thereof. This has the advantage that a better finish can be provided than if the second coating were pressed into the pores of the paper.

While I have illustrated herein diagrammatically a machine for carrying out my invention, yet I wish to state that the invention is not limited to any particular mechanism.

I claim:

1. The process of producing a smooth glazed surface on paper which consists in applying to the surface of the paper a main coating of the finishing material which produces the desired smooth glazed surface, 8 forcing said material into the pores of the paper and spreading said material evenly over the surface of the paper, partially drying said material, passing the partially-dried coated face of the paper over a smooth-surfaced roll which rotates at the same surface speed as the speed at which the paper moves and at the same time causing the coated face of the paper to be pressed lightly against the roll whereby any wavy formation resulting 9 from the partial drying operation is eliminated, then spraying onto the coated face of the partially dried paper a second coating of the same material as that of the first coating, and then drying the paper in any usual 10 way.

2. The process of coating paper for the purpose of producing a smooth glazed surface thereon which consists in applying to a moving web of paper a primary coating of 11 material adapted to produce a hard, smooth, glazed surface, forcing said coating into the pores of the paper, and spreading said coating evenly over the paper, subjecting the coated paper to the action of drying 12 blasts of air whereby the coating is partially dried, smoothing the partially dried coated surface of the paper to eliminate any wavy formation produced by the partial drying, and then applying to the partially dried coated face of the paper a light, evenly-spread second coating of the same material as that comprising the first coating and then drying the paper in any usual way.

3. The process of coating paper which 13 consists in applying to the paper a primary coating of finishing material adapted to produce a smooth, glazed surface on the paper, partially drying said coating by subjecting it to the action of drying blasts 14 of air, smoothing the coating while in its partially dried state so as to eliminate any wavy formation produced in the drying op-

eration, and then spraying a second coating of the same finishing material onto the primary coating.

4. The process of coating paper which consists in applying to the paper a primary coating of finishing material adapted to produce a hard, glazed surface, forcing said coating into the pores of the paper, partially but not completely drying said coat-

ing by subjecting it to the action of drying 10 blasts of air, spraying a second coating of the same finishing material onto the partially dried surface of the paper and then drying the paper in any usual way.

In testimony whereof I have signed my 15 name to this specification.

CHARLES M. GAGE, Jr.